

I. S. FRANKLIN.

VEHICLE BODY AND METHOD OF MAKING THE SAME.

APPLICATION FILED APR. 18, 1919.

1,362,249.

Patented Dec. 14, 1920.

2 SHEETS—SHEET 1.



INVENTOR:  
Ira S. Franklin  
By Right Brain Quinby May  
ATTY:

I. S. FRANKLIN.

VEHICLE BODY AND METHOD OF MAKING THE SAME.  
APPLICATION FILED APR. 18, 1919.

1,362,249.

Patented Dec. 14, 1920.

2 SHEETS—SHEET 2.

FIG. 8.



FIG. 9.



FIG. 10.



INVENTOR:

Ira S. Franklin  
Lytle Brown Lumby May  
ATTYS.

# UNITED STATES PATENT OFFICE.

IRA S. FRANKLIN, OF BOSTON, MASSACHUSETTS.

## VEHICLE-BODY AND METHOD OF MAKING THE SAME.

1,362,249.

Specification of Letters Patent. Patented Dec. 14, 1920.

Application filed April 18, 1919. Serial No. 291,111.

To all whom it may concern:

Be it known that I, IRA S. FRANKLIN, citizen of the United States, residing at Boston, in the county of Suffolk and State 5 of Massachusetts, have invented new and useful Improvements in Vehicle-Bodies and Methods of Making the Same, of which the following is a specification.

This invention relates to the seat-containing body of a vehicle such as an automobile, 10 a body of this character presenting an external surface of considerable area and having a smooth and lustrous finish.

The object of the invention is to enable 15 a body having all the desirable characteristics of the metal and wooden bodies in general use, to be produced without the extensive use of these materials, and at less expense than heretofore, and to provide a 20 body capable of being more easily and inexpensively repaired than heretofore in case its external surface is punctured or fractured.

The invention consists in the improvements 25 which I will now proceed to describe and claim.

Of the accompanying drawings forming a part of this specification,—

Figure 1 is a perspective view of an automobile body constructed in accordance with 30 my invention.

Fig. 2 is a section on line 2—2 of Fig. 1.

Fig. 3 is a perspective view of the sill forming an element of the body shown by 35 Figs. 1 and 2.

Fig. 4 is a perspective view of a former adapted for use in making the wall or curb portion of the body.

Fig. 5 is a transverse section showing the 40 former in place in the body.

Fig. 6 is an enlarged fragmentary section on line 6—6 of Fig. 2.

Fig. 7 is an enlarged fragmentary section on line 7—7 of Fig. 1.

Fig. 8 is a perspective view showing the 45 sill provided with reinforcing members.

Fig. 9 is a perspective view of the sill shown by Fig. 8, and a wall or curb formed thereon.

Fig. 10 is a fragmentary perspective view, 50 showing a portion of the sill, portions of

the reinforcing members shown by Figs. 8 and 9, supplemental reinforcing members, and portions of the wall, door openings being formed in the latter.

55

The same reference characters indicate the same parts in all of the figures.

Referring first to Figs. 1 to 7 of the drawings, 12 represents a frame-shaped sill, and 13 represents a frame-shaped wall or curb, 60 united at its lower edge portion to the sill, said parts being formed to constitute the seat-containing and floor-supporting body of an automobile. In making the sill I employ any suitable paper board, such as the 65 well known binders board, preferably about one-eighth or three-sixteenths of an inch thick. Said material is absorbent, so that the cementitious material hereinafter described sinks into the surfaces of strips cut 70 from the material. This material is cut into strips of any suitable length, and about four inches wide, and these are assembled side-by-side, and suitably bent to form a laminated frame-shaped sill. Before the 75 strips are assembled they are treated with a hard-drying cementitious material capable of penetrating the surfaces of the strips, of firmly uniting the strips, and of solidifying by drying and thus rendering the strips 80 and the entire sill extremely hard and rigid. A suitable cementitious material may be made as follows:

Dissolve in water one pound of casein and one and one-half ounces of borax. 85 Then make a composition consisting of five and one-third ounces of formaldehyde 40° Baumé, and eight ounces of ammonia 28° strength. When this composition effervesces it is added to the casein and borax 90 composition, the whole being thoroughly mixed.

The paper board strips are immersed in a bath of the cementitious material above described, until the material penetrates the 95 surfaces of the strips, after which the strips are assembled and pressed together. In assembling the strips they are bent into frame shape around a suitable former, the length of the strips being such that their ends 100 meet to form a joint 14, which is preferably at the forward end of the sill, as shown

by Fig. 3. The said ends may be caused to adhere to each other by the cementitious material.

In making the wall 13 I employ sheets 5 of flexible absorbent material considerably thinner and wider than the sill strips, and assemble the same side-by-side to form a laminated frame-shaped wall. I prefer to alternate sheets of textile fabric, such as 10 open-mesh cheese cloth, or gunny cloth, with sheets of kraft paper, or other absorbent paper of about the thickness of ordinary wrapping paper.

The sheets are saturated with the cementitious material above described, the latter being preferably heated, and are then wrapped one at a time around a former 16, placed upon the sill 12, each sheet being drawn tightly and its ends meeting to form 15 a joint 17 (Fig. 6). I prefer to first apply a layer of textile fabric, then a layer of paper, then another layer of textile fabric, then another layer of paper, and so on until a wall of sufficient thickness is built up. 20 Usually about eight layers constitute a sufficient number. The lower edges of the layers overlap the outer edge of the sill, as shown by Figs. 2 and 5, and may be united to the sill by the cementitious material alone, or 25 by said material and screws, or other suitable fasteners.

After the completion of the wall, the former is removed, leaving the body in the condition shown by Figs. 1 and 2. When 35 the cementitious material dries, the layers and the entire laminated wall become hard and rigid, and the wall is adapted to be finished in any suitable way to impart a smooth and lustrous surface.

40 The usual door openings may be provided by cutting out the portions 19 of the sides of the wall indicated by dotted lines in Fig. 1, at any suitable stage of the operation.

The wall may now be finished as follows: 45 Apply to the wall surfaces to be finished a coating 20, (Figs. 6 and 7) composed of a mixture of the described cementitious material and finely powdered talc, having the consistency of thin paste, and add to a quart 50 of this mixture about three teaspoonsfuls of silicate of soda. Several successive layers of this mixture should be applied with a brush, each layer being allowed to dry before the next is applied.

55 The described coating may be buffed, or sand-papered, to provide a smooth surface, and may then be finished by coats of paint and varnish. The coating 20 separates the finishing coat of paint and varnish from 60 the outer wall layer which backs said coating, so that the said layer is not exposed by ordinary scratches.

As shown by Fig. 6, the joints 17 are staggered or out of registration with each 65 other, so that there is no joint extending

continuously through the entire thickness of the wall, the latter being practically seamless or jointless.

Figs. 8 and 9 show the sill 12 provided with reinforcing members including upright 70 strips 22 and connecting strips 23, secured to the rear end portion of the sill and contacting with the back and with rear portions of the sides of the wall 13, upright strips 22<sup>a</sup> and 22<sup>b</sup> secured to side portions of the 75 sill, and an upright flange or dash portion 24 contacting with the front end of the wall and secured to the front end portion of the sill. The wall may be formed by wrapping the sheets or layers of which it is composed 80 around the said reinforcing members while they are supported against inward displacement, either by their own stiffness, or by a former such as the former 16.

The reinforcing members 22, 22<sup>a</sup>, 22<sup>b</sup>, 23 85 and 24, are made by assembling layers of absorbent binders board, treated with the described cementitious material, and united under pressure like the strips forming the sill. The upright reinforcing members may 90 be united to the sill by the cementitious material and by screws or bolts 26. The members 22 and 23 are preferably tongued and mortised, as shown, and united by screws or bolts 27 at their points of intersection. The 95 floor 30 of the body may be supported by the sill, as indicated by Fig. 2.

The sill 12 may be provided with supplemental reinforcing members 22<sup>c</sup> (Fig. 10), arranged to extend across the lower ends 100 of the door openings 19<sup>a</sup> formed by removing the wall portions indicated at 19 (Fig. 1).

I claim:

1. A vehicle body wall or curb composed 105 of layers constituting a laminated continuous seamless open frame, each layer being of flexible absorbent sheet material and having ends which meet to form joints, and the joints of the several layers being out of 110 coincidence with each other, so that the wall as a whole is practically jointless, and a hard-drying cementitious material absorbed by and uniting said layers and rendering 115 the wall rigid, and a rigid waterproof coating adherent to and covering the surfaces of said body, and having a finished external surface separated from the layer which backs said coating.

2. A vehicle body comprising a body wall 120 or curb, substantially as specified, and a frame-shaped floor-supporting sill united to the lower edge portion of said wall, said sill being composed of layers of fibrous flexible absorbent sheet material, and a hard-drying 125 cementitious material, which penetrates the surfaces of and unites said layers and renders the sill rigid.

3. The method of making a vehicle body wall or curb, which consists in applying 130

to sheets of flexible material a hard-drying cementitious material, wrapping said sheets around a suitable support to form a continuous laminated practically seamless open 5 frame, allowing the cementitious material to dry, and thus solidify the body, and finishing the external surfaces of said body by buffing said surfaces, applying to the

buffed surfaces a pasty waterproof coating including a hard-drying liquid adherent to 10 and penetrating the said buffed surfaces and powdered material giving body to the coating, and finally finishing said coating.

In testimony whereof I have affixed my signature.

IRA S. FRANKLIN.